

## UNITED STATES PATENT OFFICE

CAMILLE DREYFUS, OF NEW YORK, N. Y., AND GEORGE SCHNEIDER, OF EAST ORANGE, NEW JERSEY, ASSIGNORS TO CELANESE CORPORATION OF AMERICA, A CORPORATION OF DELAWARE

## TREATMENT OF FABRIC CONTAINING CELLULOSE ESTERS

No Drawing.

Application filed July 28, 1928. Serial No. 298,094.

This invention relates to the treatment of textile materials such as yarn or fabric containing organic esters of cellulose, and particularly cellulose acetate, with a paste containing an alkaline agent in such a manner that the safe ironing point of the same is appreciably increased, the textile material is rendered capable of being dyed with cotton dyes, and other of its properties are improved.

An object of our invention is to treat yarns or fabrics containing organic esters of cellulose with a pasty mass containing alkaline material in such a manner that the yarn is saponified on the surface of the filaments whereby the temperature at which the yarn or fabric may be ironed is considerably increased.

Another object of our invention is to treat textile materials containing organic esters of cellulose with a paste containing alkali in such concentration and in such a manner that the textile material may be dyed with dischargeable colors, whereby discharge prints may be readily produced on the textile material so treated. Other objects of our invention will appear from the following detailed description.

Fabrics containing organic esters of cellulose, and particularly cellulose acetate, must be ironed or calendered at a comparatively low temperature, since if the iron or calender is above about 220° C., sticking of the fabric to the same, and melting of the cellulose acetate is liable to result. Furthermore, the discharge printing on fabrics containing organic esters of cellulose to produce light figures on dark backgrounds has heretofore offered serious difficulties. This is due to the fact that the dark colors such as reds, blues and blacks that are available for the dyeing of cellulose acetate fabric cannot usually be discharged by the ordinary color discharging agents.

We have discovered that if yarns or fabrics containing organic esters of cellulose, such as

cellulose acetate, have applied thereto a pasty mass containing an alkaline agent in the manner set forth below, intense surface saponification of the filaments takes place on the surface of the yarn or filament of the organic esters of cellulose, so that a fabric is produced whose safe ironing point is raised to 250° to 260° C. or more. Moreover, the fabric when treated by our process is capable of being dyed with cotton dyes that may be discharged by printing pastes containing ordinary discharging agents.

Because of the fact that the saponification is concentrated on the surface of the filaments or yarn, the textile material produced has substantially all the desirable properties of untreated textile material containing organic esters of cellulose.

In accordance with our invention, we treat fabrics or yarn containing organic esters of cellulose with a pasty mass containing a solution of alkaline material and a thickening agent in any suitable manner. The paste may contain, if so desired, direct cotton dyes that are not affected by alkalies.

The fabric or yarn to be treated may contain any organic esters of cellulose such as cellulose acetate, cellulose formate, cellulose propionate and cellulose butyrate. The fabric to be treated may be of any desired construction; that is, it may be woven, knitted or netted. The fabric or yarn may consist wholly of one or more organic esters of cellulose or it may be a mixed material containing other fibres such as cotton and silk.

The alkaline material employed in the mass may be an alkali or an alkaline salt capable of producing hydroxyl ions in aqueous solution. Of the alkalies we have found sodium hydroxide, potassium hydroxide and ammonium hydroxide to be suitable. Examples of suitable alkaline salts are sodium carbonate, potassium carbonate, sodium phenolate, potassium phenolate, sodium silicate, potassium silicate, sodium sulphite, potas-

5 sium sulphite, trisodium phosphate or tri-potassium phosphate. Any one or a mixture of two or more of these alkaline materials may be used. In order to promote surface saponification, the paste may also contain buffer salts or modifying agents such as soap, sodium acetate, borax or ethyl alcohol. The amount of alkaline material that we prefer to employ corresponds in amount to 1 to 10% and preferably 3, 4 to 5% of caustic soda based on the weight of the pasty mass.

15 Any suitable thickening agent may be used in the paste, examples of which are gum tragacanth, gum tragasol, dextrine, British gum, water soluble cellulose ethers, starches or gum arabic. Instead of using a gelatinizable material as the thickening agent, mineral substances such as fuller's and infusorial earth may be employed, but these are not preferred.

20 The alkaline paste may be applied by printing rolls either locally but preferably over the whole surface by means of pin rolls or pad rolls in any suitable manner. The 25 paste may also be applied by brushing or spraying or by any other method for coating textile material with a paste.

25 After the composition containing the alkaline material is applied to the fabric, the 30 same is quickly dried by passing the same over heated drums, through a dryer or in any other desired manner, and the fabric may then be steamed at such temperature and for such time as to obtain the required degree of 35 saponification. The amount of alkali applied is sufficient to cause saponification of the organic ester material, say to the extent of 3% or 5% to 10% or more, up to 20%, as measured by the loss of weight the material 40 has suffered during the saponification. The fabric or yarn, after treatment by our process, has a safe ironing point of 250° to 260° C. or more and is intensely saponified on the surface. By "intense surface saponification" 45 is meant the concentration of saponification of the cellulose ester material on the surface of the yarn, while the interior of the yarn is very little affected, and, therefore, consists essentially of cellulose esters. This is indicated by the fact that when cellulose acetate 50 fabrics are treated in accordance with the above described methods, the solubility of the fabric in acetone is relatively high, and the fabric may be dyed with cotton dyes because of the fact that the surface of the yarn 55 is essentially reconstituted cellulose or approximately so.

60 The fabric, after it has been treated with the saponifying paste by any of the above methods, as above indicated, is capable of being dyed by dyestuffs that have an affinity for cellulose acetate but not for cotton, such as are known as SRA dyes, and also by dyes that have an affinity for cotton, but not for cellulose acetate, such as direct cotton dyes

and basic dyes, because of the intense surface saponification of the yarn. The direct cotton colors available for dyeing this material are within all ranges of colors. These cotton dyes include blues, blacks and reds, which may be discharged by ordinary discharge printing pastes, and therefore discharge prints of dark backgrounds may be produced on this fabric,—a result heretofore not readily attainable on fabrics containing cellulose acetate yarn.

70 The fabric, so treated and after having been dyed with direct cotton dyes, may be printed with a discharge paste which contains a reducing agent, and which may or may not contain colors for printing the discharged portions. After printing with the discharge paste, the fabric may be steamed and given other treatments as is well understood in the art.

75 The discharge paste may be applied in any suitable manner, such as by means of engraved or embossed rolls, plates or blocks. The paste may also be applied through stencils by means of brushing or spraying. The discharge paste may contain any suitable reducing agent such as sodium hydrosulphite, formaldehyde, zinc hydrosulphite, or the substances known as "protolin" which is sulphoxylate of zinc formaldehyde, etc. For 80 obtaining a white background, the sodium hydrosulphite or formaldehyde hydrosulphite are preferred, whereas if a colored discharge is desired the protolin is preferred.

85 In order further to illustrate our invention 100 the following specific example is given.

#### Example

A woven fabric consisting wholly of cellulose acetate yarn has applied thereto over its 105 entire surface either one of the following pastes.

#### Paste A

|                                      | Parts by weight |
|--------------------------------------|-----------------|
| Gum tragacanth thickening containing | 110             |
| 6% of gum tragacanth                 | 50              |
| Water                                | 40              |
| Caustic soda                         | 4               |

#### Paste B

|                                                     | Parts by weight |
|-----------------------------------------------------|-----------------|
| British gum thickening                              | 20              |
| (7 parts by weight of the gum and 5 parts of water) |                 |
| Water                                               | 10              |
| Caustic soda                                        | 0.7             |

#### Paste C

|                           | Parts by weight |
|---------------------------|-----------------|
| Gum arabic thickening 1—1 | 85              |
| Water                     | 40              |
| Caustic soda              | 4               |

125 The paste may be applied on a printing machine by means of a pin roller or an all engraved roller or by any suitable device for applying the paste to the entire surface of the fabric. The printed fabric is then imme- 130

diately passed over drying drums to dry the paste, and is then steamed for 20 minutes with steam at 5 pounds pressure. The fabric thus produced has a safe ironing point of 260° C. and has an affinity for cotton dyes as well as cellulose acetate dyes. It may be finished in any desired manner. If desired, the fabric may be dyed with direct cotton dyes and then discharged printed. It may also be printed or dyed in any desired manner.

10 It is to be understood that the foregoing detailed description is given merely by way of illustration and that many variations may be made therein without departing from the spirit of this invention.

15 Having described our invention, what we claim and desire to secure by Letters Patent is:

1. Method of increasing the safe ironing point of fabric containing organic ester of cellulose filaments comprising applying to the whole surface thereof a paste containing a thickening agent and an alkaline material in amounts to cause surface saponification of said organic ester of cellulose filaments to increase substantially the safe ironing point thereof.

2. Method of increasing the safe ironing point of fabric containing cellulose acetate filaments comprising applying to the whole surface thereof a paste containing a thickening agent and an alkaline material in amounts to cause surface saponification of said cellulose acetate filaments to increase substantially the safe ironing point thereof.

3. Method of increasing the safe ironing point of fabric containing organic ester of cellulose filaments comprising applying to the whole surface thereof a paste containing a thickening agent and an alkaline material in amounts to cause surface saponification of said organic ester of cellulose filaments to increase substantially the safe ironing point thereof and then quickly drying the same.

4. Method of increasing the safe ironing point of textile material containing organic ester of cellulose filaments comprising applying to the whole surface thereof a paste containing a thickening agent and an alkaline material in amounts to cause surface saponification of said organic ester of cellulose filaments to increase substantially the safe ironing point thereof.

5. Method of increasing the safe ironing point of textile material containing cellulose acetate filaments comprising applying to the whole surface thereof a paste containing a thickening agent and an alkaline material in amounts to cause surface saponification of said cellulose acetate filaments to increase substantially the safe ironing point thereof.

6. Method of increasing the safe ironing point of textile material containing organic ester of cellulose filaments comprising applying to the whole surface thereof a paste con-

taining a thickening agent and an alkaline material in amounts to cause surface saponification of said organic ester of cellulose filaments to increase substantially the safe ironing point thereof and then quickly drying the same.

In testimony whereof, we have hereunto subscribed our names.

CAMILLE DREYFUS.  
GEORGE SCHNEIDER.

75

80

85

90

95

100

105

110

115

120

125

130